

Patented Apr. 15, 1924.

1,490,523

# UNITED STATES PATENT OFFICE.

LOGAN G. THOMSON, OF CINCINNATI, OHIO, ASSIGNOR TO THE CHAMPION COATED PAPER COMPANY, OF HAMILTON, OHIO, A CORPORATION OF OHIO.

## PROCESS OF MANUFACTURING PAPER.

No Drawing.

Application filed March 14, 1921. Serial No. 452,259.

To all whom it may concern:

Be it known that I, LOGAN G. THOMSON, a citizen of the United States, and a resident of Cincinnati, in the county of Hamilton and State of Ohio, have invented a certain new and useful Process of Manufacturing Paper, of which the following is a full, clear, and exact description.

My invention relates to processes of imparting softness and flexibility to coated paper by incorporation into the paper of slow drying or slow solidifying material.

A considerable use has sprung up for coated paper for use in advertising circulars which are folded and mailed without protecting boards and are thus subjected to strains, which paper made from wood pulp has not been found capable of withstanding.

The requirements, so far as I am advised, have demanded a paper rich in rag content and hence expensive as compared, for example, to sulphite pulp. A sulphite paper is tinny and brittle to a certain extent and the coating or glaze thereon will crack and the body of the fibre fracture upon the folding of a circular for mailing, as in the above cited instance.

It is the object of my invention to incorporate into a sulphite or other wood pulp paper more particularly, but into any form of paper generally, what may be termed a size of a slow drying or slow solidifying substance, so that upon coating the paper, the non-drying content in the body stock will give flexibility and softness even after coating a very strong, raw stock containing a large proportion of sulphite pulp. I accomplish my process in details as will be pointed out below and duly claimed.

I make up the paper in any desired way on any machine that is used in the paper business, using preferably sulphite pulp as the main ingredient. According to one way of making the paper, I run it through the machine exactly as in the usual practice and after it is ready for coating I pass it through a process similar to the usual coating where I flow onto the paper, in the same way as the usual coating is imposed, a quantity of some slow solidifying substance, such as glycerine, or other oily substance of like character, so far as solidifying is concerned. According to one method I dissolve the glycerine in water, one part glycerine to four parts water by volume and the coating ma-

chine and subsequent drying apparatus removes the water, leaving the proper amount of glycerine.

In controlling the flow and percentage of water used with glycerine and the operation of the machine, I have used enough glycerine, for example, as to put into the paper about fourteen percent, by weight of glycerine; and I find that this glycerine will not dry out of the paper due to the drying action, above mentioned.

The paper so filled with glycerine I may then store for some days or immediately pass to a coating machine where the usual coating is added and such calendering is done as may be desired. The coating may be china-clay, or such other coating as is desired to give the wished for enamel-like or glossy surface to the paper.

According to another method I may tub size the paper with the glycerine while in the process of manufacture, as for example, in the usual Fourdrinier machine of the present time, and in this tub sizing process take such precaution as may be necessary to prevent stickiness of the paper, due to the glycerine as it passes through the final drying rolls of the machine, such as, for example, blowing the web with hot air before it strikes the next drier.

My process is regulated so as to insure the positioning within the fibrous structure of the paper of a glycerine-like substance, which paper may then be coated without destroying the soft and pliable quality.

Having thus described my invention, what I claim as new and desire to secure by Letters Patent, is:—

1. A process of forming paper, which consists in first making a web of paper, then incorporating into said web around fourteen per cent of glycerine by weight, and then coating the paper with an enamel-like coating adapted to retain the non-drying substance in the paper.

2. A process of forming paper, which consists in first making a web of paper from a large percentage of sulphite pulp, then incorporating into said web a quantity of glycerine, and then coating the paper with an enamel-like coating adapted to retain the non-drying substance in the paper.

3. A process of forming paper, which consists in first making a web of paper from a large percentage of sulphite pulp, then in-

corporating into said web around fourteen per cent of glycerine by weight and then coating the paper with an enamel-like coating adapted to retain the non-drying substance in the paper.

4. A finished paper, comprising mainly sulphite pulp formed into paper in the de-

sired way, a quantity of a relatively non-drying substance positioned within the fibrous structure of the said paper, and a coating of enamel-like nature on the surfaces of said paper.

10

LOGAN G. THOMSON.